

Patented Aug. 30, 1932

1,874,956

## UNITED STATES PATENT OFFICE

BENJAMIN GALLSWORTHY, OF BAYONNE, NEW JERSEY, ASSIGNOR TO THE TEXAS COMPANY, OF NEW YORK, N. Y., A CORPORATION OF DELAWARE

### CUTTING OIL

No Drawing.

Application filed September 30, 1930. Serial No. 485,553.

This invention relates to cutting oils.

As is well known, the office of cutting oil is to cool the cutting tool and at the same time, lubricate the face of the tool. Straight mineral oils can be used as cutting oils but the more usual and better practice is to compound the mineral oil with a fixed oil such as lard oil, sperm oil, cottonseed oil or the like. The fixed oils are used for compounding with mineral oil because such mixtures are much more adhesive and oily than straight mineral oil.

I have found that a highly satisfactory cutting oil may be made by compounding mineral oil with oxidized paraffin wax or, preferably, with that fraction of partially oxidized paraffin wax which has a melting point below 95° F., this product giving to the compounded oil the desirable quality of adhesiveness or oiliness. The oxidized wax may be subjected to sweating in the usual manner to obtain the desired fraction having a melting point of 95° F. The oxidized paraffin wax is stable and does not tend to decompose with age in the manner that animal and vegetable oils become rancid, and in this respect oxidized paraffin wax is superior to oils such as lard, sperm or cottonseed oil as the compounding agent. Furthermore, the added product is less expensive than any of the animal and vegetable oils heretofore used, and on this account the ultimate cost of the final product can be lowered.

I have found that a mineral lubricating oil having a Saybolt universal viscosity of about 100 seconds at 100° F. compounded with from 15% to 30% of oxidized paraffin wax produces a very satisfactory cutting oil. To meet the needs of large plants requiring cutting oils suitable for turning, drilling, reaming, threading, etc., it may be necessary to depart somewhat from the specifications above given and to use an oil of greater or lesser viscosity and more or less of the wax than the 15% to 30% mentioned, and I desire therefore to be limited only as indicated in the appended claims.

I claim:

1. A cutting oil consisting practically of

mineral oil compounded with from 15% to 30% of oxidized paraffin wax.

2. A cutting oil consisting practically of a relatively low viscosity mineral lubricating oil compounded with from 15% to 30% of 55 oxidized paraffin wax.

3. A cutting oil consisting practically of mineral oil compounded with from 15% to 30% of that portion of partially oxidized paraffin wax which has a melting point below 95° F. 60

In witness whereof I have hereunto set my hand this 23rd day of September, 1930.

BENJAMIN GALLSWORTHY.

65

70

75

80

85

90

95

100